



US005199253A

**United States Patent [19]****Berger****Patent Number: 5,199,253****Date of Patent: Apr. 6, 1993****[54] NYLON ROPE HAVING SUPERIOR  
FRICTION AND WEARING RESISTANCE****[75] Inventor: George A. Berger, Lafayette, La.****[73] Assignee: American Manufacturing Company,  
Inc., Lafayette, La.****[21] Appl. No.: 833,611****[22] Filed: Feb. 13, 1992**

|           |         |                       |           |
|-----------|---------|-----------------------|-----------|
| 4,263,777 | 4/1981  | Wada et al. ....      | 57/253 X  |
| 4,317,000 | 2/1982  | Ferer .....           | 174/70 R  |
| 4,405,686 | 9/1983  | Kuroda et al. ....    | 428/370 X |
| 4,412,474 | 11/1983 | Hara .....            | 87/6      |
| 4,709,544 | 12/1987 | Charvet .....         | 57/236 X  |
| 4,801,503 | 1/1989  | Jennings .....        | 57/253 X  |
| 4,929,503 | 5/1990  | Shirasaki et al. .... | 428/373   |

**Primary Examiner—John M. Jillions****Assistant Examiner—William Stryjewski****Attorney, Agent, or Firm—Louis Weinstein****Related U.S. Application Data****[63] Continuation of Ser. No. 553,883, Jul. 16, 1990.****[51] Int. Cl.<sup>5</sup> ..... D02G 3/02; D02G 3/36****[52] U.S. Cl. ..... 57/236; 57/231;  
57/237; 57/238; 57/244; 57/248; 428/370****[58] Field of Search ..... 57/230, 231, 236, 237,  
57/238, 244, 248; 428/370, 373, 374, 365****[56] References Cited****U.S. PATENT DOCUMENTS**

|           |         |                        |          |
|-----------|---------|------------------------|----------|
| 1,604,075 | 10/1926 | Reisenberg .....       | 57/230   |
| 2,134,022 | 10/1938 | Bell .....             | 57/237   |
| 2,190,854 | 2/1940  | Whitlock .....         | 57/230 X |
| 2,591,628 | 4/1952  | Snyder .....           | 57/211   |
| 3,010,275 | 11/1961 | Hartmann et al. ....   | 57/231   |
| 3,201,930 | 8/1965  | Stirling .....         | 57/230 X |
| 3,315,455 | 4/1967  | Stoller .....          | 57/231 X |
| 3,389,548 | 6/1968  | Lachaussee et al. .... | 57/244   |
| 3,415,052 | 12/1968 | Stanton .....          | 57/231   |
| 3,691,751 | 9/1972  | Hiller et al. ....     | 57/145   |
| 3,778,993 | 12/1973 | Glushko et al. ....    | 57/145   |
| 4,055,941 | 11/1977 | Rivers et al. ....     | 57/251 X |
| 4,058,049 | 11/1977 | Bech .....             | 57/202 X |

**[57]****ABSTRACT**

A multi-strand nylon rope having improved abrasion resistance comprised of a plurality of strands. Each strand is comprised of a plurality of yarns wherein each yarn is formed of a predetermined number of filaments. The filaments of each yarn are twisted together to form a yarn of a predetermined size, the twist direction being opposite that of the final ply yarn direction. For a right lay rope a sufficient number of filaments are twisted together in the left or "S" direction to produce a yarn of a predetermined size. Three or more yarns prepared in this manner are then plied or twisted together in the opposite or right direction. The cover for each strand is formed of alternate yarns of standard and oblong filaments, respectively, the oblong filaments having a modification ratio of three, forming a rope having increased abrasion resistance, a hand and feel that is not stiff or unmanageable and which resists strand-to-strand wet abrasion.

**20 Claims, 3 Drawing Sheets**



*Fig. 1b*

*Fig. 1a*

13

Fig. 2b

Fig. 2a



*Fig. 3*



*Fig. 4*

## NYLON ROPE HAVING SUPERIOR FRICTION AND WEARING RESISTANCE

This is a continuation of application Ser. No. 5 07/553,883, filed Jul. 16, 1990.

### FIELD OF THE INVENTION

The present invention relates to rope, and more particularly, to multiple strand nylon rope, each strand being formed of a plurality of yarn and having alternating cover yarns of first and second types respectively formed of filaments which have round and oblong cross-sections.

### BACKGROUND OF THE INVENTION

The present invention relates to cordage, and more particularly, to an improved rope made of nylon.

Nylon ropes have been in use for many years. Nylon is known to provide strong, elastic rope fibers. Rope formed of nylon provides excellent shock absorption, withstanding dynamic loads that have been found to break other ropes. Nylon has good resistance to abrasion, rot, mildew, marine growth, petroleum products, and most chemicals and is widely used in the marine industry as anchor, mooring, shock and towing lines. Nylon rope construction is typically produced in three or four strand twisted, eight strand plaited and solid braid and are satisfactory in most applications.

Nevertheless, nylon ropes experience significant 30 wearing due to wet abrasion. More particularly, abrasion caused by contact of the rope with another surface such as a bollard, cleat or other metal surface is accelerated when the nylon rope is wet.

Techniques for protecting the rope against wearing have included coating the rope or applying another covering such as a canvas or leather sleeve. These techniques are unsatisfactory since they increase production costs of the rope and further tend to affect the stiffness and hand of the rope.

### BRIEF DESCRIPTION OF THE INVENTION

The present invention is directed to providing a rope which significantly increases the resistance of rope and particularly nylon rope to abrasion with the structure of said rope being characterized by comprising strands which are twisted together wherein each strand is formed of a plurality of twisted yarns. A first group of yarns comprise the core of a strand while a second group of yarns collectively form a cover for the strands. The core yarns and alternating ones of the cover yarns encircling the core yarns are formed of substantially the same filaments. The remaining alternating yarns forming the strand cover are each comprised of obround filaments.

For a right lay rope the yarns are twisted in the left or "S" direction. Three or more such yarns are then plied, or twisted together in the opposite or right (i.e. "Z") direction.

The yarns are then placed in a rope machine and positioned to produce a strand. The strands are then twisted together in the "Z" direction to form a multi-strand rope.

The cover yarns formed of obround filaments provide an abrasion resistance superior to that of the round filaments. However, the obround filaments are stiff and would otherwise form unmanageable rope if the cover yarns were made of 100 percent obround filaments.

A cover layer constructed employing alternating yarns respectively formed of round and obround filaments yields a rope having increased abrasion resistance compared with ropes containing only round filaments; a hand or feel that is not stiff and unmanageable; and increased resistance to strand-to-strand wet abrasion as well as surface wearing.

In the preferred embodiment, the rope is formed of nylon filaments of round and obround construction.

### OBJECTS OF THE INVENTION

It is, therefore, one object of the present invention to provide a novel rope structure formed of strands having a novel cover layer adapted to significantly increase the wet abrasion resistance of the rope.

Still another object of the present invention is to provide a novel rope structure comprised of a plurality of twisted strands wherein each strand is provided with yarns forming a cover layer wherein alternating yarns of the cover layer for the yarns forming the core of each strand are respectively formed of different filaments.

Still another object of the present invention is to provide a novel rope structure comprised of a plurality of twisted strands wherein each strand is provided with 25 yarns forming a cover layer for the yarns forming the core of each strand wherein alternating yarns of the cover layer are respectively formed of different filaments wherein said filaments are respectively round and obround.

Still another object of the present invention is to provide a nylon rope having a novel construction for yielding excellent wet abrasion resistance in which the twisted strands of the rope are each formed of a plurality of twisted yarns, and having a cover layer of twisted 30 yarns wherein alternating yarns of the cover layer are respectively formed of different nylon filaments.

Still another object of the present invention is to provide a nylon rope having a novel construction for yielding excellent wet abrasion resistance in which the 35 twisted strands of the rope are each formed of a plurality of twisted yarns, and having a cover layer of twisted 40 yarns wherein alternating yarns of the cover layer are respectively formed of different nylon filaments.

Still another object of the present invention is to provide a nylon rope having a novel construction for yielding excellent wet abrasion resistance in which the 45 twisted strands of the rope are each formed of a plurality of twisted yarns, and having a cover layer of twisted 50 yarns wherein alternating yarns of the cover layer are respectively formed of different nylon filaments.

### BRIEF DESCRIPTION OF THE FIGURES

The above, as well as other objects of the present invention will become apparent when reading the accompanying description and drawings, in which:

FIG. 1a shows a longitudinal view of a section of three strand twisted rope embodying the principles and design structures of the present invention;

FIG. 1b shows a cross-sectional view of the rope of 55 FIG. 1a;

FIG. 2a shows a longitudinal view of a section of an eight strand braided rope embodying the principles of the present invention;

FIG. 2b shows a cross-sectional view of the rope of FIG. 2a; and

FIGS. 3 and 4 show sectional views of two types of filaments utilized in the construction of the ropes of FIGS. 1b and 2b.

### DETAILED DESCRIPTION OF THE INVENTION

FIGS. 1a and 1b show a three strand twisted rope 10 embodying the principles of the present invention.

Rope 10 is comprised of three strands S1, S2 and S3 which are all substantially identical in design and are twisted together in the "Z" direction as shown in FIG. 1a.

1a. For this reason, the construction of only one of the strands will be described herein for purposes of brevity.

Strand S1 is comprised of a plurality of yarns of first and second types. Yarns Y1, shown shaded, are utilized as cover yarns for strand S1. Yarns Y2 form the center or core of the strand as well as serving as a cover yarn. The yarns Y1 and Y2 forming the cover yarns are arranged in alternating fashion and surround the core yarns Y2 in the manner shown in FIG. 1b.

In the preferred embodiment, two different nylon fibers (i.e. filaments) with different cross-sections are utilized for constructing rope 10.

The yarns Y2, in the preferred embodiment, are formed of either "standard" industrial nylon or 192 filament/1260 denier nylon. A sufficient number of the filaments are twisted together to produce a yarn of a predetermined size with the filaments being twisted in the direction opposite that of the final ply yarn direction. Three or more such yarns are then plied or twisted together in the opposite direction. For example, when forming a right lay rope the filaments of a yarn are twisted in the left or "S" direction. Three or more such 25 yarns are then plied or twisted together in the opposite or right (i.e. "Z") direction.

The Y1 yarns, which are only used to form the cover yarns for each strand, are preferably formed of a nylon identified by the trademark "HYTEN" manufactured 30 by DuPont. These yarns are prepared in a manner similar to the preparation of the standard nylon yarn. Filaments of a predetermined size or denier are twisted together. The twist direction is the same as that employed for the standard nylon yarns. Once the single 35 yarns are prepared they are grouped and plied or twisted together in the opposite or right direction.

The filaments of the standard nylon have a circular cross-section as shown in FIG. 4. The filaments employed in the strands Y1 are obround as shown in FIG. 40. 3. The obround filaments, which have flat parallel sides and round ends, preferably have a modification ratio (i.e. width to thickness) which is of the order of 3.0. The filaments employed to form the yarns Y2 are preferably a standard 1260 denier, 192 filament. The obround filaments are produced in deniers from 2000 to 6000.

After preparation of the yarns Y1 and Y2 in the manner described hereinabove, they are then placed in a rope machine in order to produce a strand similar to those shown in FIG. 1b. The strands Y1 and Y2 formed in the manner described hereinabove are placed in a rope machine (not shown for purposes of simplicity) and positioned to produce a rope such as shown in FIG. 1b wherein a plurality of Y2 strands form the core or inner portion of the strands S1-S3. The strand cover is 55 comprised of alternating yarns Y1 and Y2.

Each of the strands S1, S2 and S3 are substantially identical to one another and are twisted together in the "Z" direction (to form a right lay rope).

FIG. 2 shows an eight strand braided rope 20 embodying the principles of the present invention and comprised of eight strands S1 through S8, each strand formed of yarns Y1 (shown shaded) and Y2 which are formed in a manner similar to the yarns Y1 and Y2 in the embodiment 10 of FIGS. 1a and 1b.

Although the preferred embodiments shown herein are three strand and eight strand braided rope, it should be understood that other conventional structures may

be utilized such as twelve strand and double braid nylon rope, while employing the principles of the present invention.

5 Nylon rope embodying the principles of the present invention exhibit the characteristics of increased abrasion resistance as compared with conventional nylon ropes, a hand and feel that is not stiff or unmanageable and excellent resistance to strand-to-strand wet abrasion.

10 A latitude of modification, change and substitution is intended in the foregoing disclosure, and in some instances, some features of the invention will be employed without a corresponding use of other features. Accordingly, it is appropriate that the appended claims be construed broadly and in a manner consistent with the spirit and scope of the invention herein described.

15 What is claimed is:

1. A rope formed of only synthetic fibers exhibiting excellent resistance to wet abrasion comprising:

a plurality of strands, each strand including a core portion and a cover portion; said core portion being comprised of a plurality of 20 yarns of a first type, each yarn being formed of a plurality of filaments formed of nylon; said cover portion being comprised of a plurality of 25 yarns of said first type and a plurality of yarns of a second type, each yarn of said second type being formed of a plurality of filaments formed of nylon, said first and second type yarns being arranged in alternating fashion about said core portion; said filaments in said first type of yarn having a first cross-sectional, non-circular, shape for providing 30 said first type of yarn with greater abrasion resistance than said second type of yarn and said filaments in said second type of yarn having a second cross sectional shape different from said first cross sectional shape for providing said second type of 35 yarn with a greater flexibility than said second first type of yarn.

2. The rope of claim 1 wherein said strands are 40 twisted together.

3. The rope of claim 2 wherein rope is comprised of 45 at least three strands.

4. The rope of claim 1 wherein said first type of 50 yarns comprise a number filaments sufficient to provide a 1260 denier nylon yarn.

5. The rope of claim 1 wherein the second type of 55 filaments are nylon and each filament has a denier in the range from 2000 to 6000.

6. The rope of claim 1 wherein each yarn is formed by 60 twisting a predetermined number of filaments; a plurality of said twisted filaments being twisted together to form a yarn.

7. The rope of claim 6 wherein said yarns are 65 arranged to form a strand of substantially circular cross-section comprised of a cover layer of yarns defining a substantially circular cover surrounding the remaining yarns making up each strand.

8. The rope of claim 7 wherein the filaments twisted together are twisted in a first direction and wherein the groups of twisted filaments are twisted in a direction opposite said first direction.

9. The rope of claim 1 wherein providing the second 65 type of yarn with greater abrasion resistance is obtained by providing the filaments of said first type of yarn with a round cross-sectional shape and wherein providing the second type of yarns with a greater flexibility is

obtained by providing the filaments of said second type of yarn with an obround cross-sectional shape.

10. The rope of claim 9 wherein said obround filaments have a modification (M) of three (3) wherein M is represented as the ratio of the length of each filament relative to its thickness which length and thickness directions are measured in the cross-sectional direction.

11. A rope according to claim 1 wherein the plurality of filaments forming said first type of yarn are twisted.

12. A rope according to claim 1 wherein the plurality of filaments forming said second type of yarn are twisted.

13. A rope according to claim 1 wherein the filaments of said first type of yarn have a round cross-sectional shape and the filaments of said second type of yarn have an obround cross-sectional shape. 15

14. The rope of claim 1 wherein said 1260 denier nylon yarn is comprised of the order of 192 filaments. 20

15. The rope of claim 1 wherein the denier of said filaments of said second type of yarn is greater than the denier of the filaments of said first type of yarn. 25

16. The rope of claim 15 wherein the denier of the filaments of said second type of yarn is at least 300 times greater than the denier of the filaments of said first type of yarn. 30

17. The rope of claim 15 wherein the thickness of the filaments of said second type of yarn is at least 300 times greater than the thickness of the filaments of said first type of yarn. 35

18. The rope of claim 15 wherein the denier of the filaments of said second type of yarn is between 333 and 1000 times greater than the denier of the filaments of said first type of yarn.

19. The rope of claim 1 wherein the thickness of said filaments of said second type of yarn is greater than the thickness of the filaments of said first type of yarn.

20. An all nylon rope especially adapted for use in marine applications and exhibiting excellent resistance to wet abrasion comprising:

a plurality of strands, each strand including a core portion and a cover portion;  
said core portion being comprised of a plurality of yarns of a first type, each first type of yarn being formed of a plurality of twisted filaments of a first type;  
said cover portion being comprised of a plurality of yarns of said first type and a plurality of yarns of a second type, each second type of yarn being formed of a plurality of twisted filaments of a second type said first and said second type yarns being arranged in alternating fashion about said core portion to surround said core portion;  
said filaments in said first type of yarn having a round cross-section for providing said first type yarns with a greater flexibility than said second type of yarn and said filaments of said second type of yarn having an obround cross-section for providing said second type of yarns with greater abrasion resistance than said first type of yarn.

\* \* \* \* \*

UNITED STATES PATENT AND TRADEMARK OFFICE  
CERTIFICATE OF CORRECTION

PATENT NO. : 5,199,253

DATED : April 6, 1993

INVENTOR(S) : Berger

It is certified that error appears in the above-identified patent and that said Letters Patent is hereby corrected as shown below:

Column 1, line 11, change "yarn" to --yarns--

Column 2, line 19, after "layer" insert --for the yarns  
forming the core of each strand--

Column 2, lines 20-21, delete "for the yarns forming the  
core of each strand"

Signed and Sealed this

Twenty-eighth Day of December, 1993

Attest:



BRUCE LEHMAN

Attesting Officer

Commissioner of Patents and Trademarks